# EUROPEAN PATENT SPECIFICATION

(11) **EP 1 994 125 B1**
(45) Date of publication and mention of the grant of the patent: **17.10.2012**
(21) Application number: 07718024.8
(22) Date of filing: 12.01.2007
(51) Int. Cl.: C10M 163/00, C10N 10/04, C10N 10/12, C10N 30/02, C10N 30/04, C10N 30/06, C10N 30/10, C10N 30/12, C10N 40/25, C10N 60/14

(54) **LOW SULFUR, LOW ASH AND LOW PHOSPHOROUS LUBRICANT COMPOSITION**
SCHMIERMITTELZUSAMMENSETZUNG MIT GERINGEM SCHWEFEL-, GERINGEM ASCHE- UND GERINGEM PHOSPHORGEHALT
COMPOSITION DE LUBRIFIANT À FAIBLES TENEURS EN SOUFRE, CENDRES ET PHOSPHORE

(30) Priority: 13.01.2006 US 758840 P; 09.01.2007 US 651185
(43) Date of publication of application: 26.11.2008
(62) Divisional of application: 12182716.6
(73) Proprietor: ExxonMobil Research and Engineering Company, Annandale, NJ 08801-0900 (US)
(72) Inventor: BUCK, William, H., West Chester, PA 19382 (US); FARNG, L., Oscar, Lawrenceville, NJ 08648 (US); DECKMAN, Douglas, E., Mullica Hill, NJ 08062 (US); GIVENS, Jr., Willie, A., Dumfries, VA 22026 (US); HORODYSKY, Andrew, G., Cherry Hill, NJ 08003 (US)
(74) Representative: Troch, Geneviève
(86) International application number: PCT/US2007/000915
(87) International publication number: WO 2007/084407

(56) References cited:
- WO-A1-96/29381
- GB-A- 1 032 008
- US-A1- 2002 035 042
- US-A1- 2003 013 620
- US-A1- 2005 288 194

## Description

### BACKGROUND OF THE INVENTION

### Field of the Invention

This invention relates to lubricating oil compositions suitable for use in internal combustion engines. More particularly, this invention relates to a low ash, sulfur, and phosphorous lubricating oil composition.

### Background

Many means have been employed to reduce overall wear and friction as well as to control oxidation/cleanliness in modern engines, particularly automobile engines. The primary reasons include prolonging engine life by reducing engine wear and increasing the resistance to oxidation by reducing the engine's sludge/deposit through degradation. Many of the solutions to reducing wear have been strictly mechanical including building engines with wear resistant parts, modifying the contact geometry and adding special coating materials. Other solutions to improve cleanliness involve the use of metal containing detergents. Recently, considerable work has also been done with lubricating oils to enhance their anti-wear/anti-oxidation properties by modifying them with ashless antioxidants and anti-wear components.

Contemporary lubricants such as engine oils use mixtures of additive components. Examples of additives components include, anti-wear and extreme pressure components, fuel economy improving components, friction reducers, dispersants, detergents, inhibitors and viscosity index improving additive. These additives provide energy conservation, engine cleanliness and durability and high performance levels under a wide range of performance conditions including temperature, pressure and lubricant service life. For example WO 96/29381 discloses lubricant and fuel compositions containing a combination of a ring-substituted diphenyl sulfide, a succinic type dispersant and a zinc dithiophosphate having superior antiwear and extreme pressure properties as well as corrosion resistance and high temperature cleanliness.

Throughout the world, legislation aimed at reducing automotive emissions is pushing down the level of sulfur in fuels. Recently, lubricants are coming under scrutiny as a source of air pollution and emission catalyst deactivation. Phosphorus is known to be poisonous to automotive three-way HC conversion catalysts. Sulfur is known to be poisonous to deNox catalysts and zinc/moly phosphates are key contributors to cause plugging of the exhaust particulate filters. The sulfur, ash and phosphorous components are commonly referred to as "SAP" or "SAPS" in the art. Accordingly, there is a need for a low sulfur, ash, and phosphorous component additive for lubricating oils that provides favorable performance properties.

Conventional engine oil technology relies heavily on zinc dithiophosphate ("ZnDTP" or "ZDDP"). ZnDTP is a versatile, anti-wear/anti-oxidant component that provides extremely low cam and lifter wear and favorable oxidation protection under severe conditions. ZnDTP is disadvantageous, especially at high treat rates. The major problem with ZnDTP is the poisoning effects to after-treatment devices that may aggravate emission problems. In addition, ZnDTP has strong interactions with dispersants, detergents, other anti-wear components and MoDTC causing antagonistic effects on friction, sludge and deposit, if inappropriate concentrations are utilized. Replacing ZnDTP additives is not a simple endeavor since the wear protection demand for today's engine is extremely high and extremely rigorous chemical limits on ZnDTP.

Based on the above, there is a need for the development of a low phosphorus, low sulfur and low ash lubricating oil and additive with low levels of ZnDTP. Accordingly, this invention satisfies that need.

### SUMMARY OF THE INVENTION

A lubricating oil composition is disclosed. This composition, comprises a lubricating oil basestock, an alkylated diphenyl sulfide of at least 0.01 and less than 20 weight percent of the composition, a dispersant-detergent-inhibitor system of less than 15 percent weight percent of the composition, a zinc dithiophosphate additive of at least 0.1 weight percent of the composition and no more than 1.0 weight percent of the composition, the composition having less than 630 PPM phosphorus, less than 710 PPM zinc, less than 5,000 PPM sulfur, less than 8 TBN, less than 1.0 weight percent ash and the dispersant-detergent-inhibitor system comprising a dispersant chosen from borated and non-borated succinimides, succinic acid-esters and succinic acid-amides, alkylphenol-polyamine coupled Mannich adducts and combinations thereof and a detergent chosen from calcium phenates, calcium sulfonates, calcium salicylates, magnesium phenates, magnesium sulfonates, magnesium salicylates, metal carbonates, borated detergents and combinations thereof.

### BRIEF DESCRIPTION OF THE DRAWING

Figure 1 illustrates the viscosity increase profiles for a Group V base stock with different additive embodiments.

### DETAILED DESCRIPTION OF THE INVENTION

This invention relates to engine lubricants formulated with functional fluids and/or additives and compositions. The composition of the invention is a low ash, sulfur, phosphorus engine lubricant compositions comprising oils of lubricant viscosity containing a minor amount of multi-functional anti-wear/anti-oxidation additive. The anti-wear/anti-oxidation additive is an alkylated diphenyl sulfide.

The lubricating oil compositions according to the invention maintain low frictional properties of film under various operating conditions and favorably maintain sufficiently high film thickness at high operating temperatures to provide a minimum lubricant film to protect against wear at a variety of temperatures.

The lubricating oil compositions further maintains cleanliness over the entire range of operating conditions while reducing wear to an absolute minimum and provides favorable oxidation and corrosion control, under the most severe operating conditions.

Traditionally, antiwear and extreme pressure additives have been chosen from zinc dithiophosphates, phosphites, sulfurized olefins/esters, sulfur-nitrogen additives and similar components. Friction reducers have been chosen from molybdenum additives including Moly dithiocarbamates ("MoDTC"), Molydithiophosphates ("MoDTP"), and other organic moly-containing compounds), amines, amides and similar components. Metal detergents have been chosen from calcium or magnesium phenates, sulfonates, salicylates, carbonates and similar components. Antioxidants have been chosen from hindered phenols, arylamines, dihydroquinolines, phosphites and thiol/thiolester/disulfide/trisulfide compounds. These additives are rich in sulfur, phosphorus and/or ash content as they form strong chemical films to the metal surfaces.

Diphenyl sulfide, diphenyl oxide, biphenyl, diphenylmethane, and many other related analogs are utilized as heat transfer fluids since they are stable materials that can resist thermal stress under severe conditions. conditions. However, the direct use of the non-alkylated aromatics in lubricants are relatively limited to low concentrations due to the limited compatibility with other hydrocarbon base stocks.

Alkylated aromatics, especially sulfur containing alkylated aromatics have been developed by applying alkylation technique to functional or non-functional aromatics providing good thermal-oxidative stability while maintaining good compatibility. These alkylated aromatics have excellent compatibility with other base oils and superb solvency and stability making them unique synthetic oils including Group V or functional fluids. U.S. Patent Nos. 5,105,042, and 5,177,284 disclose the process conditions of making alkylated naphthalenes. US. Patent Nos. 5,372,734, 5,552,071, 5,371,248, and 5,286,396 disclose the preparation of alkylated benzothiophene-derived lubricants, alkylated diphenyl ether lubricants, alkylated benzofuran-derived lubricants and alkylated phenoxathins for lubricants.

The prior art literature referenced above fails to disclose the use of alkylated aromatics in a low SAP environment with high quality base stocks. In addition, the prior art fails to disclose the favorable anti-wear/anti-oxidation properties and unexpected, superb cleanliness features which make the alkylated aromatics functional fluids suitable for low ash and low phosphorus engine oils. In different embodiments the preferred degree of alkylation varies ranging from mono- to di- to multiple alkylates. However, mono-alkylates are more desirable than others. The desired carbon to sulfur and oxygen ratio is in a range from 10:1 1 to 400:1 on atomic basis with a more preferred range of 20:1 to 200:1 and an even more preferred range of 25:1 to 100:1.

In one embodiment, lubricating oils, especially synthetic oils, when blended with low level of zinc dithiophosphates and/or optionally molybdenum friction modifiers can provide substantial reductions in wear and oxidation. These combinations provide improvements in engine service life and durability with excellent overall performance benefits. In addition, these combinations typically minimize deleterious effects such as instability, undesirable high viscosity, high friction, deposits and the like, when added to lubricating oils. Combinations of alkylated aromatics with low level of sulfur-free detergents such as, salicylates, ashless phenols and arylamines, and boron containing additives, and any combination thereof further provide synergies.

According to the invention, novel highly stable, sulfur containing, alkylated aromatics have been synthesized and evaluated as functional fluids and/or additives for lubricants including low ash, sulfur, phosphorus engine lubricants. The novel compositions possess multi-functional anti-wear/anti-oxidation/cleanliness/friction reducing-fuel economy properties. In addition, these combinations can improve the wear protection of most lubricants used in both automotive and commercial diesel engine applications, while maintaining desirable viscometrics. In this embodiment, the composition is favorable suited for low ash passenger car engine oils. When used as Group V base stocks including functional fluids or co-base stocks, the typical alkylated aromatic concentration is in the range of 0.1 to 20 wt%, preferably 0.5 to 8 wt%.

This invention is referred to as a low ash, sulfur and phosphorus engine oil formulated with extremely stable, sulfur functional fluids selected from alkylated diphenyl sulfides.

Preferably, the highly stable engine oil fluids has a very low viscosity of less than 20 cSt at 400°C, with fully saturated structures with an Iodine value less than 1, low volatility of less than 15 wt% loss in Noack and even more preferably high resistance to oxidation/thermal breakdown. The most preferred embodiment provides favorable viscometrics for engine oils since fuel economy is heavily influenced by viscometrics. A variety of alkylated diphenyl sulfides are suitable for this invention. For example, ADPS-1 is an experimental synthetic fluid made by the alkylation of diphenyl sulfide with long chain alkenes over the USY catalyst.

The lubricant compositions, besides being built around the alkylated diphenyl sulfide, also contain low levels of zinc, phosphorus and sulfur components and dispersant-detegent-inhibitor system comprising a dispersant chosen from borated and non-borated succinimides, succinic acid-esters and succinic acid-amides, alkylphenol-polyamine coupled Mannich adducts and combinations thereof and a detergent chosen from calcium phenates, calcium sulfonates, calcium salicylates, magnesium phenates, magnesium sulfonates, magnesium salicylates, metal carbonates, borated detergents and combinations thereof.
Persons skilled in the art will recognize the ability to include additives that favorably enhances lubricant performance including anti-friction, anti-oxidation and anti-wear performance while successfully meeting the stringent wear, oxidation and cleanliness performance requirements in modem engines. Examples of suitable additives include but are not limited phenolic and aminic ashless anti-oxidants, high and low levels of metal detergents, molybdenum or organic friction modifiers, defoamants, seal swell additives, pour point depressants including contemporary DDI additive packages, and any combination thereof.

In some embodiments, we have discovered that these new synergistic combination has favorably improved lubricant performance parameters while maintaining excellent compatibility to exhaust after-treatment devices. The core of the preferred embodiment comprises stable sulfur containing functional fluid and a significantly reduced amount of ZnDTP and metal detergents, and optionally enhanced amount of ashless anti-oxidants and friction modifiers. The resulting formulation provides an engine oil lubricant with less than 630 PPM phosphorus, less than 710 PPM zinc, less than 5,000 PPM sulfur, less than 8 TBN, less than 1.0 wt% ash and high nitrogen/zinc or nitrogen/phosphorus ratios. In one embodiment, the general formulation of the low SAP engine oil containing the alkylated aromatics is summarized in Table 1.

**Table 1**

| Component Type | Wt% | Elements in Formulated Oils (ppm) + Other Restrictions |
|---|---|---|
| Sulfur aromatic | 0.01 - 20.0% | < 4500 ppm sulfur, volatility <10 |
| functional fluid/additive | | wt% |
| Zinc dithiophosphate additive | 0.1 - 1.0% | 100 - 630 ppm phosphorus, 105-710 ppm zinc |
| Dispersant-detergent-inhibitor system | <15.0% | <1800 ppm nitrogen, <1.0 wt ash, TBN <8, N/P >1 (wt/wt) N/Zn >1 (wt/wt) |
| Molybdenum additive | 0-2.0% | <210 ppm molybdenum |
| Boron additive | 0-8.0% | <400 ppm boron |

These components can be used with a variety of base stocks, including group I, II, III, IV, and V, and GTL as well as a variety of mixtures thereof. However, due to other performance requirements including volatility, stability, viscometrics, and cleanliness feature, premium engine oils prefer to use group II and higher ("Group II+") base oils to ensure that they can achieve desirable overall performance levels as well as maximizing the full potential of the unique synergies among additives. Additional significant synergies were identified among alkylated aromatics and Group II+ high performance base stocks including Group II, III, IV, V, VI or GTL base stocks.

Base stocks having a high paraffinic/naphthenic and saturation nature (>90 wt%) can often be used advantageously in certain embodiments. Such base stocks include Group II and/or Group III hydroprocessed or hydrocracked base stocks, or their synthetic counterparts such as polyalphaolefin oils, GTL or similar base oils or mixtures of similar base oils.

In a preferred embodiment, at least about 20% of the total composition should consist of such Group II or Group III base stocks or GTL, with at least about 30% being preferable, and more than about 80% on being most preferable. Gas to liquid base stocks can also be preferentially used with the components of this invention as a portion or all of the base stocks used to formulate the finished lubricant. We have discovered, favorable improvement when the components of this invention are added to lubricating systems comprising primarily Group II, Group III and/or GTL base stocks compared to lesser quantities of alternate fluids.

Dispersants include borated and non-borated succinimides, succinic acid-esters and amides, alkylphenol-polyamine coupled Mannich adducts and any combination thereof. In some embodiment, it can often be advantageous to use mixtures of such above described dispersants and other related dispersants. Examples include additives that are borated, those that are primarily of higher molecular weight, those that consist of primarily mono-succinimide, bis-succinimide, or mixtures of above, those made with different amines, those that are end-capped, dispersants wherein the back-bone is derived from polymerization of branched olefins such as polyisobutylene or from polymers such as other polyolefins other than polyisobutylene, such as ethylene, propylene, butene, similar dispersants and any combination thereof.

Detergents include calcium phenates, calcium sulfonates, calcium salicylates, magnesium phenates, magnesium sulfonates, magnesium salicylates, metal carbonates, borated detergents, and any combination thereof. The detergents can be neutral, mildly overbased, or highly overbased.

The antioxidants include hindered phenols, arylamines, low sulfur peroxide decomposers and other related components. Inhibitors and antirust additives may be used as needed. Seal swell control components and defoamants may be used with the mixtures of this invention. Various friction modifiers may also be utilized. Examples include but are not limited to amines, alcohols, esters, diols, triols, polyols, fatty amides, various molybdenum phosphorodithioates (MoDTP), molybdenum dithiocarbamates (MoDTC), sulfur/phosphorus free organic molybdenum components, molybdenum trinuclear components, and any combination thereof.

ZnDTP is widely utilized for providing anti-wear protection to modern engine oils with few other components sharing similar functions. As the levels of ZnDTP are reduced, the wear protection must rely on a new anti-wear system. Preferably, that new anti-wear system will be low in ash, sulfur and substantially free of phosphorus components to provide favorable performance with the new exhaust systems. Typically, the sulfur-containing alkylated aromatics possess moderate level of highly stable, less volatile sulfur, that is different from the volatile sulfur liberated from zinc dithiophosphates. Therefore, these sulfur-containing alkylated aromatics are harmless to exhaust after-treatment devices but effective in protecting engine parts against wear mechanism.

In one embodiment, the principle advantage of this new invention is the synergistic combination of multi-functional, alkylated sulfur aromatics and small amount of zinc dithiophosphate additives that favorably provides oxidation, corrosion, seal stability and frictional properties. Even more important is the ability to provide anti-wear protection with lower levels of sulfur, phosphorus and zinc in the engine oil formulations are significantly less than that typically used in today's engine oils. Another principle advantage of this invention is the unique combination of alkylated sulfur aromatics with boron-containing additives for superb cleanliness features, such as the effective control of undercrown deposit formation. Another principle advantage in one embodiment is the synergistic combination of alkylated sulfur aromatics and low level of sulfur-free metal detergents including calcium and magnesium salicylates and carbonates. An additional synergistic combination is an alkylated sulfur aromatics with ashless anti-oxidants to improve oxidation protection and extended drain intervals. Another potential advantage is the unique combination embodiment of alkylated sulfur aromatics with friction reducers to improve fuel economy.

### Examples

Table 2 below discloses bench and tribology testing data for alkylated diphenyl sulfide (experimental sample "ADPS-1") in Passenger Vehicle Engine Oils.

**Table 2**

| Lubricant Example | | 1 | 2 | 3 |
|---|---|---|---|---|
| ADPS-1 =93-59386 | | | | 4% ADPS-1 |
| | | 1.0% ZnDTP | 0.5% ZnDTP | 0.5% ZnDTP |
| 01-60665 = 0% P EO | | 99% 01-60665 | 99.5% 01-60665 | 95.5% 01-60665 |
| Phosphorus, % | | 0.10 | 0.05 | 0.05 |
| Sample Number | | 02-713 | 02-714 | 02-33611 |
| Solubility Appearance | | C&B | C&B | C&B |
| 4 Ball Wear | WSD (mm) | 0.44 | 0.48 | 0.42 |
| 40Kg/1200rpm/60min./200 F | K Factor | 1.11 | 1.62 | 0.78 |
| 4 Ball EP (D2783) | LNS (Kg) | 80 | 80 | 100 |
| 30C/10sec./1760rpm | Weld Ld (Kg) | 200 | 200 | 200 |
| | LWI | 35.1 | 34.5 | 41.7 |
| Cu Corrosion (D130-9) | 24 hrs/250F | 1A | 1A | 1A |
| PDSC (Ramp 10C/min) | Onset T (C) | 232 | 229.7 | 235.1 |
| 288° C, 16hrs Tube Rating (1 = Clean) | | 3.8 | 3.5 | 3.3 |
| | | | | |
| HFRR 0.7Kg/60Hz/0.5mm/ | Scar X/Y (mm) | 0.317/0.7 | 0.3/0.767 | 0.26/0.70 |
| 60min./75C | Calc. Sc. Area | 0.174 | 0.181 | 0.147 |
| | | | | |
| D2896 | TBN | 4.27 | 4.23 | - |
| D874 (wt%) | Sulfated Ash | 0.53 | 0.38 | 0.35 |
| D6443 (wt%) | Phosphorus | 0.1003 | 0.0507 | 0.0497 |
| D6443 (wt%) | Zinc | 0.1118 | 0.0577 | 0.0572 |
| D6443 (wt%) | Calcium | 0.0329 | 0.0332 | 0.0317 |
| D6443 (wt%) | Magnesium | 0.0595 | 0.0496 | 0.0482 |
| D6443 (wt%) | Copper | <0.002 | <0.002 | <0.002 |
| D6443 (wt%) | Chlorine | 0.0047 | 0.0049 | 0.0048 |
| D6443 (wt%) | Sulfur | 0.2799 | 0.1783 | 0.4761 |

The base formulation (01-60665) is a phosphorus-free, partially formulated engine oil with Group III base stocks, ashless antioxidants, ashless dispersants, metal detergents, defoamants, viscosity modifiers and other performing components.

As illustrated in the above Table 2, very good anti-wear, anti-oxidation and corrosion control can be achieved with sulfur-derived alkylated aromatics in the low P passenger vehicle lubricants ("PVL"). As shown in the High Frequency Reciprocating Rig ("HFRR") and Four-Ball EP wear test, the functional fluids formulated low SAPS engine oils can help to improve anti-wear properties evidenced by the low wear scar areas and wear coefficients ("K Factor") measured.

In addition, there are synergistic benefits of low SAP additives with Group II and higher base stocks. The synergistic benefits include favorable cleanliness, wear properties, catalyst compatibility and oxidation.

Comparing lubricant example 1 by adding 1000 ppm phosphorus and lubricant example 2 by adding 500 ppm phosphorus, noticeable anti-wear performance differences can be seen, which are believed to be directly affected by ZnDTP concentrations. Typically, the more ZnDTP, the better anti-wear protection. However, when 4% alkylated diphenyl sulfide was added to make lubricant example 3, which has the same level of 500 ppm phosphorus as lubricant example 2, a significant 19% reduction of wear scar areas and an observed 52% reduction in wear coefficients was measured.

The Table 2 results for lubricant example 3 are even better when compared to lubricant example 1. In the presence of more ZnDTP, for example 1000 ppm P in lubricant example 1 versus 500 ppm P in lubricant example 2, a reduction of calculated scar area from 0.18 mm² to 0.174 mm² is expected. However, a significant reduction to 0.147 mm² range for lubricant example 3 is an unexpected result.

In the Four-Ball EP test, lubricant example 3 also demonstrated superb load carrying property as evidenced by the higher last non-seizure load of 100 kg and a greater Load Wear Index of 41.7 when compared to lubricant examples 1 and 2. The improvement in Load Wear Index from lubricant examples 2 to lubricant examples 3 is almost 21 %. The high temperature stability of lubricant example 3 is also shown by the Pressured differential Scanning Calorimetry ("PDSC") data on ramping method. Comparing lubricant examples 2 to 3, the onset temperature is raised from 229.7°C to 235.1°C respectively providing 54% better oxidation control, assuming the oxidation rates doubled with every 10 °C increase in temperature. Therefore, lubricant example 3 could provide 54 % better oxidation resistance than lubricant 2 if we quantify the control by viscosity or acid value increases or any other measurements.

The hot tube test is also used to assess cleanliness features of engine oils under high temperature oxidation conditions. As exhibited in Table 2, lubricant example 3 has slightly better cleanliness result than both lubricant examples 1 and 2 as the lower the rating, the better the cleanliness. This data illustrates that more ZnDTP reduces lubricant cleanliness as lubricant example 1 has the worst result as ZnDTP is known to decompose to various species at elevated temperatures. The copper corrosion results indicated that adding ADPS to the engine oil formulations causes no adverse impact to their copper corrosivity. Adding ADPS will certainly increase the sulfur content of the engine oil. However, the final sulfur level of 0.476 wt% for lubricant example 3 is still under the current ILSAC GF-4 standard of 0.5 wt%. In conclusion, exceptionally good oxidative stability and low wear in low phosphorous engine oils can be achieved by using alkylated sulfur aromatics such as, ADPS thus providing favorable performance properties suitable for modem engine oils.

The outstanding anti-oxidation/anti-wear performance is further verified by another set of Four-ball EP and hot tube tests. Table 3 is a Table similar to Table 2 comparing lubricant examples 1 and 2 from Table 2 with additional lubricant example tests. As shown in the Table 3 data, when the low phosphorus engine oil was formulated with extremely low level of ZnDTP such as, 0.025 wt% phosphorous, the last non-seizure load dropped to 63 kg and the load wear index also dropped to 28.2 comparing table 4 lubricant example 4 versus lubricant examples 2 and 1. This is clearly not desirable as poor EP performance indicates weak load carrying property. Adding a conventional sulfur EP additive, Rhein-Chemie's RC-2411™, could not improve the load carrying property significantly as shown in lubricant example 5. However, as shown in example 6, adding 2 wt% of ADPS to the base engine oil formulation provides significant improvement.

**Table 3**

| Lubricant Example | | 1 | 2 | 4 | 5 | 6 |
|---|---|---|---|---|---|---|
| Funct'lized fluids or cobase oil | | | | | | 2% ADPS-1 |
| | | 1% ZnDTP | 0.5% ZnDTP | 0.25% ZnDTP | 0.25% ZnDTP | 0.25% ZnDTP |
| 01-60665 = 0% P EO | | 99% 01-60665 | 99.5% 01-60665 | 99.75%01 -60665 | 99.5%01-60665 | 97.5%01-60665 |
| | | | | | 025%RC24 11 | 025%RC2 411 |
| | | (0.10% P) | (0.05% P) | 0.025% P | 0.025% P | 0.025% P |
| Sample Number | | 02-713 | 02-714 | 02-31205 | 02-35335 | 02-35333 |
| Solubility/ Appearance | | C&B | C&B | C&B | C&B | C&B |
| 4 Ball EP (D2783) | LNS (Kg) | 80 | 80 | 63 | 63 | 80 |
| 30C/10sec./17 60rpm | Weld Ld (Kg) | 200 | 200 | 200 | 200 | 250 |
| | LWI | 35.1 | 34.47 | 28.21 | 28.41 | 36.16 |
| Cu Corrosion (D130-8) | 3hrs/ 210F/H2O | 1A | 1B | 1A | 1B | 1B |
| Cu Corrosion (D130-9) | 24 hrs/250F | 1A | 1A | 2A | 2B | 2A |
| 288° C, 16hrs Tube Rating (1 = Clean) | | 3.8 | 3.5 | | 2.8 | 2.8 |
| | | | | | | |

| D2896 | TBN | 4.27 | 4.23 | 5.45 | 4.11 | 5.59 |
|---|---|---|---|---|---|---|
| D874 (wt%) | Sulfated Ash | 0.53 | 0.38 | 0.33 | 0.33 | 0.32 |
| D6443 (wt%) | Phosphorus | 0.1003 | 0.0507 | 0.0244 | 0.0245 | 0.0246 |
| D6443 (wt%) | Zinc | 0.1118 | 0.0577 | 0.0287 | 0.0278 | 0.028 |
| D6443 (wt%) | Calcium | 0.0329 | 0.0332 | 0.0331 | 0.0331 | 0.0325 |
| D6443 (wt%) | Magnesium | 0.0595 | 0.0496 | 0.0505 | 0.0501 | 0.0514 |
| D6443 (wt%) | Copper | <0.002 | <0.002 | <0.002 | <0.002 | <0.002 |
| D6443 (wt%) | Chlorine | 0.0047 | 0.0049 | 0.0048 | 0.005 | 0.0049 |
| D6443 (wt%) | Sulfur | 0.2799 | 0.1783 | 0.124 | 0.1463 | 0.2988 |

RC-2411™ is an aliphatic sulfur additive, which has even higher sulfur content than the ADPS used in lubricant example 6 of table 3. Some sulfur-containing additives, including aliphatic sulfur species, could provide equivalent favorable antiwear/extreme pressure performance as alkylated sulfur aromatics providing that they are thermally stable and non-corrosive. However, many sulfur-containing aliphatic sulfur additives, used by themselves alone, are not sufficient to provide anti-wear protection while maintaining satisfactory anti-corrosion properties as demonstrated in example 4 and 5 of table 3. Lubricant example 6 (with levels of 0.025 wt% phosphorus) of table 3 illustrates the last non-seizure load and the load-wear index improved to be equivalent to or better than the lubricant example 1 with levels of 0.1 wt% phosphorus engine oil. In addition, the weld load increased to 250 kg when comparing lubricant example 6 to lubricant example 1. Lubricant example 6 shows a synergistic benefits of using an ADPS aliphatic sulfur compound with group II and higher base stock.

These results are exceptional favorable in the presence of additive treat level of ADPS. As stated before, the hot-tube test is used to measure the relative cleanliness of engine oils with the higher the rating on the scale form 1 to 9, the dirtier the lubricant. Lubricant example 6, ADPS formulated oil, demonstrated better cleanliness than oils with higher levels of ZnDTP including lubricant examples 1 and 2. As shown in table 3 for lubricant example 5, the total sulfur of the ADPS containing formulation is below the ILSAC GF-4 requirements.

Figure 1 illustrates the viscosity increase profiles for a Group V base stock with different additive embodiments. Reference numerals 11 and 12 represent viscosity increase profiles for two runs for 7 wt% alkylated naphthanates additives. Reference numeral 13 represents viscosity increase profiles for 7 wt% of TMP ester and 14 represents a viscosity increase profile for 7% dibasic acid ester (adipate ester). Finally, the reference numerals 15 and 16 represent viscosity increase profiles for 7 wt% and 1 wt% ADPS additive respectively.

Figure 1 demonstrates that alkylated sulfur aromatics 15 and 16 can provide favorable performance advantages in oxidation control versus other group V synthetic fluids in the presence of equal amount of ashless anti-oxidants. This performance benefit was shown using the ExxonMobil Research Catalytic Oxidation Test ("ERCOT"). In the ERCOT test, 50 ppm of soluble iron is added to 100g of test fluid. The fluid is heated at 165°C while air is bubbled through the sample at a rate of 1L/hour. The kinematic viscosity at 40°C of the catalyzed oil is monitored as a function of time. When the antioxidants in the fluid are consumed, a significant increase in viscosity is observed. The base engine oil formulation has about 450 ppm phosphorus from reduced ZnDTP, and a total of 1.0 wt% hindered phenol and alkylated arylamine ashless anti-oxidants. In the presence of 7 wt% experimental ADPS-1, the oil induction time has been increased by 70-80 hours in the ERCOT test. Even present in just 1 wt% ADPS, the oil induction time can still be 40-50 hours longer than synthetic esters or alkylated naphthalenes. Therefore, Figure 1 illustrates the strong synergy of ADPS with an ashless anti-oxidant.

Another important performance feature of the current invention is after-treatment compatibility. To measure after-treatment compatibility, a series of engine oil samples were prepared where each sample contained a single sulfur containing species as shown in Table 4. Thus, the fully formulated engine oils studied contained only the single source of sulfur listed in Table 4. Secondary ZDDP, Primary ZDDP, Thiadiazole, Sulfur-phenol, sulfurized olefin, and ADPS were studied. These fully formulated engine oils contain typical non-sulfur containing performance additives such as hindered phenols, alkylated arylamines, ashless dispersants, metal and ashless detergents, friction modifiers, defoamants, corrosion inhibitors, copper passivators, pour point depressants and seal swell agents. The single sulfur containing species in Table 4 were the last components added. Samples were volatilized at 250°C for 15 minutes using D 5800 and a comparison of the percent sulfur lost between the new oil and the oil remaining at the end of the volatilization test was made. In a direct comparison of Table 4, primary and secondary zinc dithiophosphates volatized at 12.0% and 37.0% respectively. Commercial sulfur-containing antioxidants volatized at 6.1 %, thiadiazole at 21.8%, molybdenum dithiocarbamate at 12.7%, and sulfurized olefin additive at 10.5%. ADPS exhibited extraordinarily low volatility at 2.0%. This data provides strong evidence for the favorable low emission performance benefit of using ADPS in engine oils. In this embodiment, the invention provides favorable benefit in sustaining the useful life of the after-treatment system by identifying a method to reduce volatile sulfur species to the exhaust system.

**Table 4**

| 15 Minute D5800 Sulfur Volatilization Study | |
|---|---|
| | Sulfur Volatilized, % |
| 2° ZDDP | 37.0 |
| Thiadiazole | 21.8 |
| Moly Dithiocarbamate | 12.7 |
| 1° ZDDP | 12.0 |
| Sulfurized Olefin | 10.5 |
| Sulfur Phenol* | 6.1 |
| ADPS | 2.0 |

All alkylated aromatics dissolved easily in engine oils and remained clear and bright on the shelf at ambient temperatures over period of six months or longer. Apparently, the stability of alkylated sulfur aromatics-containing oils is satisfactory and they cause no adverse effects to compatibility in the presence of other commonly used additives in engine oil compositions.

Besides unique, synergistic additive effects, it is evidenced that other highly refined, low sulfur Group II/III based oils including both hydro-processed oils and HDP as well as other Group IV/V synthetic base oils can be used to achieve favorable lubricant performance.

In summary, in one embodiment, we have discovered a new class of low sulfur, low ash and low phosphorous ("SAP") engine oils with favorable oxidation and wear protection based on alkylated sulfur-containing aromatics. This offers an effective way to reduce the amount of ZnDTP for contemporary engine oils while maintaining excellent wear, friction and oxidation performance as well as meeting stringent emission requirements. This embodiment further provides favorable synergisms to similar formulations comprising alkylated sulfur aromatics, base oils of less than 300 ppm sulfur, low levels of ZnDTP wherein the ZnDTP contributes less than 630 ppm phosphorus and/or less than 710 ppm zinc, sulfur containing additives and molybdenum containing additives.

## Claims

1. A composition having less than 630 ppm phosphorus, less than 710 ppm zinc, less than 5,000 ppm sulfur, less than 8 TBN and less than 1.0 weight percent ash, comprising:
a. a lubricating oil basestock;
b. from 0.01 to less than 20 wt.% of the composition of an alkylated diphenyl sulfide;
c. less than 15 wt.% of a dispersant-detergent-inhibitor system comprising a dispersant chosen from borated and non-borated succinimides, succinic acid-esters and succinic acid-amides, alkylphenol-polyamine coupled Mannich adducts and combinations thereof and a detergent chosen from calcium phenates, calcium sulfonates, calcium salicylates, magnesium phenates, magnesium sulfonates, magnesium salicylates, metal carbonates, borated detergents and combinations thereof; and
d. from 0.1 to 1.0 wt. % of the composition of a zinc dithiophosphate additive.

2. The composition of claim 1, further comprising a molybdenum additive wherein the molybdenum additive is less than 2 weight percent of the composition.

3. The composition of claim 1, further comprising a boron additive wherein the boron additive is less than 8 weight percent of the composition.

4. The composition of claim 1, wherein the composition has a viscosity less than 20 cSt at 400 °C, fully saturated structures with an iodine value less than 1 and a volatility less than 15 weight percent loss in Noack.

5. The composition of claim 1, wherein the alkylated aromatic concentration is at least 0.5 weight percent and no more than 8 weight percent of the composition.

6. The composition of claim 1, further comprising additives chosen from the group comprising phenolic and aminic ashless anti-oxidants, molybdenum or organic friction modifiers, defoamants, seal swell additives, pour point depressants, and any combination thereof.

7. The composition of claim 1, wherein the base stock is chosen from the group consisting of group II base stocks, group III base stocks, group IV base stocks, and group V base stocks, gas-to-liquids base stocks, and any combination thereof.

8. The composition of claim 1, wherein the alkylated aromatic additive is a mono-alkylate comprising a carbon and oxygen atomic ratio of at least 10:1 and less than 400:1.

9. The composition of claim 1, further comprising an aliphatic sulfur additive.

## Patentansprüche

1. Zusammensetzung mit weniger als 630 ppm Phosphor, weniger als 710 ppm Zink, weniger als 5.000 ppm Schwefel, einer TBN von weniger als 8 und weniger als 1 Gew.-% Asche, die:
a. Schmierölbasismaterial,
b. 0,01 bis weniger als 20 Gew.-%, bezogen auf die Zusammensetzung, alkyliertes Diphenylsulfid,
c. weniger als 15 Gew.-% Dispergiermittel-Detergenz-Inhibitorsystem, das Dispergiermittel ausgewählt aus borierten und nicht borierten Succinimiden, Bernsteinsäureestern und Bernsteinsäureamiden, Alkylphenol-Polyamin-gekoppelten Mannichaddukten und Kombinationen davon und Detergenz ausgewählt aus Calciumphenolaten, Calciumsulfonaten, Calciumsalicylaten, Magnesiumphenolaten, Magnesiumsulfonaten, Magnesiumsalicylaten, Metallcarbonaten, borierten Detergenzien und Kombinationen davon umfasst, und
d. 0,1 bis 1 Gew.-%, bezogen auf die Zusammensetzung, Zinkdithiophosphatadditiv umfasst.

2. Zusammensetzung nach Anspruch 1, die ferner Molybdänadditiv umfasst, wobei das Molybdänadditiv weniger als 2 Gew.-% der Zusammensetzung ausmacht.

3. Zusammensetzung nach Anspruch 1, die ferner Boradditiv umfasst, wobei das Boradditiv weniger als 8 Gew.-% der Zusammensetzung ausmacht.

4. Zusammensetzung nach Anspruch 1, wobei die Zusammensetzung eine Viskosität von weniger als 20 cSt bei 400°C, vollständig gesättigte Strukturen mit einem Iodwert von weniger als 1 und eine Flüchtigkeit von weniger als 15 Gew.-% Verlust gemäß Noack hat.

5. Zusammensetzung nach Anspruch 1, wobei die Konzentration an alkylierten Aromaten mindestens 0,5 Gew.-% beträgt und nicht mehr als 8 Gew.-% der Zusammensetzung beträgt.

6. Zusammensetzung nach Anspruch 1, die ferner Additive ausgewählt aus der Gruppe umfassend phenolische und aminische aschefreie Antioxidantien, Molybdän- oder organische Reibungsmodifizierungsmittel, Entschäumer, Dichtungsquellungsadditive, Stockpunktsenkungsmittel und jedwede Kombination davon umfasst.

7. Zusammensetzung nach Anspruch 1, wobei das Basismaterial ausgewählt ist aus der Gruppe bestehend aus Gruppe II-Basismaterialien, Gruppe III-Basismaterialien, Gruppe IV-Basismaterialien und Gruppe V-Basismaterialien, Gas-to-Liquid-Basismaterialien und jedweder Kombination davon.

8. Zusammensetzung nach Anspruch 1, wobei das alkylierte aromatische Additiv ein Monoalkylat mit einem Kohlenstoff-zu-Sauerstoff-Atomverhältnis von mindestens 10 : 1 bis weniger als 400 : 1 ist.

9. Zusammensetzung nach Anspruch 1, die ferner aliphatisches Schwefeladditiv umfasst.

## Revendications

1. Composition comportant moins de 630 ppm de phosphore, moins de 710 ppm de zinc, moins de 5 000 ppm de soufre, un indice de base total (TBN) inférieur à 8 et moins de 1,0 pour cent en poids de cendre, comprenant:
a. une matière de base d'huile lubrifiante;
b. de 0,01 à moins de 20 %, en poids de la composition, d'un sulfure de diphényle alkylé;
c. moins de 15 % en poids d'un système dispersant-détergent-inhibiteur comprenant un dispersant choisi parmi les succinimides boratés et non boratés, les esters d'acide succinique et les amides d'acide succinique, les adduits de Mannich couplés à une alkylphénolpolyamine et leurs combinaisons et un détergent choisi parmi les phénates de calcium, les sulfonates de calcium, les salicylates de calcium, les phénates de magnésium, les sulfonates de magnésium, les salicylates de magnésium, les carbonates métalliques, les détergents boratés et leurs combinaisons; et
d. de 0,1 à 1,0 %, en poids de la composition, d'un additif dithiophosphate zinc.

2. Composition selon la revendication 1, comprenant en outre un additif à base de molybdène dans laquelle l'additif à base de molybdène représente moins de 2 pour cent en poids de la composition.

3. Composition selon la revendication 1, comprenant en outre un additif à base de bore dans laquelle l'additif à base de bore représente moins de 8 pour cent en poids de la composition.

4. Composition selon la revendication 1, dans laquelle la composition possède une viscosité inférieure à 20 cSt à 400 °C, des structures entièrement saturées ayant un indice d'iode inférieur à 1 et une volatilité inférieure à 15 pour cent en poids de perte selon Noack.

5. Composition selon la revendication 1, dans laquelle la concentration en aromatique alkylé est d'au moins 0,5 pour cent en poids et n'est pas supérieure à 8 pour cent en poids de la composition.

6. Composition selon la revendication 1, comprenant en outre des additifs choisis dans le groupe comprenant les antioxydants sans cendres phénoliques et aminiques, les modificateurs de frottement à base de molybdène ou organiques, les antimoussants, les additifs de gonflement des joints, les agents abaissant le point d'écoulement, et une combinaison quelconque de ceux-ci.

7. Composition selon la revendication 1, dans laquelle la matière de base est choisie dans le groupe constitué par les matières de base du groupe II, les matières de base du groupe III, les matières de base du groupe IV et les matières de base du groupe V, les matières de base pour transformation de gaz en liquide, et une combinaison quelconque de celles-ci.

8. Composition selon la revendication 1, dans laquelle l'additif aromatique alkylé est un mono-alkylate comportant un rapport atomique carbone/oxygène au moins égal à 10:1 et inférieur à 400:1.

9. Composition selon la revendication 1, comprenant en outre un additif à base de soufre aliphatique.
